

## 1

3,717,578

## ANNULAR MAGNET CORE BUILT UP FROM A SOFT MAGNETIC FERRITE MATERIAL AND METHOD OF MANUFACTURING THE SAME

Nicolaas Petrus Slijkerman and Cornelis Jacobus Esveldt, Emmasingel, Eindhoven, Netherlands, assignors to U.S. Philips Corporation, New York, N.Y.

No Drawing. Continuation of abandoned application Ser. No. 831,762, June 9, 1969. This application May 27, 1971, Ser. No. 147,656

Claims priority, application Netherlands, June 8, 1968, 6808112

Int. Cl. C04b 35/26

U.S. CL. 252—62.61

3 Claims

## ABSTRACT OF THE DISCLOSURE

Annular ferrite cores having an outside diameter not exceeding 0.6 mm. and an inside diameter of at least half of the outside diameter as memory cores in electronic computers having a composition expressed in molar percentages of the ferrite-forming oxides within the following range: 74.5–80.0 mol percentage  $Fe_2O_3$ ; 12.5–14.6 mol percent  $Li_2O$ ; 3.0–8.0 mol percent  $ZnO$ ; and maximally 6.1 mol percent  $NiO$ .

These cores have pulse characteristics which are substantially temperature-insensitive over an extensive temperature range, and are responsive to comparatively weak current pulses.

In the manufacture of these magnet cores they are cooled, after heating, to room temperature at a substantially constant speed.

This application is a continuation of application Ser. No. 831,762, filed June 9, 1969, now abandoned.

It is known to use annular magnet cores built up from a soft magnetic ferrite material as memory elements in electronic computers. For these memory elements a large "speed," that is to say a very short switching time, is one of the principal requirements for use. The "switching time" ( $t_s$ ) is to be understood to mean the time which elapses between the instant at which the current intensity of the reading pulse ("test current") has risen to an amount of 10% of its maximum value and the instant at which the voltage pulse induced in the reading wire has fallen to an amount of 10% of its maximum value. The smaller the dimensions of the memory element, at a much lower control current a sufficient low value of the switching time is reached, that is to say, the element is more economical to use.

For various applications of memory elements it is also important that their pulse characteristics show substantially constant values over a large temperature range.

The memory elements according to the invention which have an outside diameter of not exceeding 0.6 mm., and an inside diameter of at least half of the outside diameter are distinguished in that at a test current,  $I_t$ , not exceeding 750 ma.:

- (a)  $t_s$ , the switching time, is smaller than 0.25  $\mu$ sec.—
- (b)  $uV_1$ , i.e. the maximum value of the output voltage upon reading of an undisturbed "one" signal which is caused by the first reading pulse, is at least 40 mv.;
- (c) the quotient

$$\frac{uV_1}{dV_z}$$

(where  $dV_z$  is the maximum value of the output voltage of a "zero" signal interfered frequently with an interfering writing pulse) at an interference ratio of 0.61

## 2

has a value of at least 3.5; "interference ratio" is to be understood to mean the value of the quotient

$$\frac{I_{pt}}{I_t}$$

of an interference-test pulse,  $I_{pt}$  and a full test pulse,  $I_t$ ; (d) in the temperature range between 0° C. and 60° C. a control current compensation not exceeding 1.9 ma./° C. is sufficient. "Control current compensation" is to be understood to mean the decrease of the test current (in ma.) necessary to maintain the output voltage at the same value at an increase of the temperature by 1° C.

15 The range of compositions of the magnet cores according to the invention is characterized by the following percentages of the metal oxides involved in forming the ferrite material, namely iron oxide, lithium oxide, zinc oxide and, if desirable, nickel oxide: 74.5–80.0 mol. percent  $Fe_2O_3$ ; 12.5–14.6 mol. percent  $Li_2O$ ; 3.0–8.0 mol. percent  $ZnO$ ; and up to 6.1 mol. percent  $NiO$ .

The preparation of the magnet cores according to the invention is preferably carried out as follows. The new materials, usually the above-mentioned metal oxides which, however, may individually be replaced partly or entirely by other compounds of the relative metals which upon heating are converted into the corresponding metal oxides, are ground in a ball mill for approximately 4 hours and at the same time mixed. The dried mixture is prefired in a fluidized bed furnace after which the prefired product is cooled and ground to a very fine powder in the course of approximately 16 hours. This powder is the suspended in acetone, while adding a binder, after which the suspension is atomized in a heated space. The resulting granules are compressed to rings of the desired dimensions which rings are sintered after removing the binder by heating at approximately 300° C. The prefired powder may alternatively be mixed with a binder to form a paste and this paste may be evenly smeared on a supporting foil 25 consisting of a suitable synthetic resin in a layer of the desirable thickness and may then be left to dry thereon, after which the ferrite layer is detached from the supporting foil and rings of the desired dimensions are punched from it, which rings are sintered again after removing the binder by heating at approximately 300° C.

The sintering of the rings is preferably carried out as follows: A number of rings are provided in a platinum boat and this is arranged within one minute, preferably in approximately 30 seconds, in the hottest region of a 30 furnace where a temperature between 1100° C. and 1200° C. prevails. The boat with the rings is kept in said region for 1½ to 8 minutes and is then pulled out of the furnace gradually at a substantially constant speed so that the rings are cooled to room temperature in a period of time varying from 5 to 25 minutes preferably within 8 to 20 minutes. The principal pulse characteristics are then measured in the resulting rings. The interference ratio used in the measurements is always 0.61.

In order that the invention may be readily carried into effect, a few examples thereof will now be described in greater detail.

## EXAMPLE I

The composition of the starting mixture was as follows:

|           | Mol percent |
|-----------|-------------|
| $Fe_2O_3$ | 74.6        |
| $Li_2O$   | 12.3        |
| $ZnO$     | 7.6         |
| 70 $NiO$  | 5.5         |

For sintering the rings (which have an outside diameter

of approximately 0.5 mm. and an inside diameter of approximately 0.3 mm.) the rings were arranged in a platinum boat in the hottest region of a furnace in a period of time of approximately 30 seconds in which region a temperature prevailed of 1105° C. Two minutes later the boat with the rings was pulled out of the furnace at a substantially constant speed. Twenty minutes afterwards the rings were cooled to room temperature.

The results of the measurements performed in the resulting magnet cores are stated in the stable after Example V. In addition to the measured values of the above-defined quantities the measured values of the quantities  $rV_1$  and  $t_p$ ,  $rV_1$  which is to be understood to means the maximum value of the output voltage upon reading a "one" signal frequently interfered with an interfering-reading pulse which is caused by the second reading pulse also recorded in the table. The peak time,  $t_p$ , is to be understood to means the period between the instant at which the current intensity of a full reading pulse has increased to an amount of 10% of its maximum value and the instant at which the output voltage caused by said pulse reaches its maximum value.

#### EXAMPLE II

The composition of the starting mixture was as follows:

|                                | Mol percent |
|--------------------------------|-------------|
| Fe <sub>2</sub> O <sub>3</sub> | 79.04       |
| Li <sub>2</sub> O              | 14.51       |
| ZnO                            | 5.00        |
| NiO                            | 1.45        |

The rings (which have an outside diameter of approximately 0.5 mm. and an inside diameter of approximately 0.3 mm.) were sintered mainly according to the prescription of Example I, with the difference that the temperature in the hottest region of the furnace now was 1169° C. The sintering time was again 2 minutes. Then the boat with the rings was pulled out of the furnace at a substantially constant speed in such manner that the rings were

#### 4 EXAMPLE IV

The composition of the starting mixture was as follows:

|                                | Mol percent |
|--------------------------------|-------------|
| Fe <sub>2</sub> O <sub>3</sub> | 77.21       |
| Li <sub>2</sub> O              | 13.61       |
| ZnO                            | 3.13        |
| NiO                            | 6.05        |

The rings had an outside diameter of approximately 0.4 mm. and inside diameter of approximately 0.25 mm. The rate of heating was again approximately 30 seconds. In the hottest furnace region temperature of 1165° C. prevailed. The rings were kept in said region for 2 minutes. Then the boat with the rings was pulled out of the furnace at a substantially constant speed, so that in a period of time of approximately 8 minutes they were cooled to room temperature.

The measured results of the resulting rings are again recorded in the table after Example V.

#### EXAMPLE V

The composition of the starting mixture was as follows:

|                                | Mol percent |
|--------------------------------|-------------|
| Fe <sub>2</sub> O <sub>3</sub> | 76.12       |
| Ni <sub>2</sub> O              | 13.06       |
| ZnO                            | 5.01        |
| NiO                            | 5.81        |

The rings had an outside diameter of approximately 0.5 mm. and an inside diameter of approximately 0.3 mm. The rate of heating was again approximately 30 seconds. A temperature of 1170° C. prevailed in the hottest furnace region. The rings were kept in said region for 2 minutes. Then the boat with the rings was pulled out of the furnace at a substantially constant speed, so that after a period of approximately 12 minutes they were cooled to room temperature.

The measured results of the resulting rings are recorded in the following table.

TABLE

| Magnet cores<br>according to<br>example number | $I_t$<br>(milli-<br>amperes) | $uV_1$<br>(milli-<br>volts) | $rV_1$<br>(milli-<br>volts) | $dV_2$<br>(milli-<br>volts) | $t_s$<br>(micro-<br>seconds) | $t_p$<br>(micro-<br>seconds) | $\frac{uV_1}{dV_2}$<br>between 0° C.<br>and 60° C.<br>(mA per ° C.) |      |
|------------------------------------------------|------------------------------|-----------------------------|-----------------------------|-----------------------------|------------------------------|------------------------------|---------------------------------------------------------------------|------|
| I                                              | 725                          | 45.3                        | 38.6                        | 12.8                        | 0.182                        | 0.098                        | 3.5                                                                 | 1.85 |
| II                                             | 725                          | 44                          | 39.7                        | 10                          | 0.208                        | 0.110                        | 4.4                                                                 | 1.7  |
| III                                            | 725                          | 42                          | 38                          | 10                          | 0.210                        | 0.110                        | 4.2                                                                 | 1.5  |
| IV                                             | 700                          | 42                          | 38                          | 9.5                         | 0.170                        | 0.100                        | 4.4                                                                 | 1.4  |
| V                                              | 725                          | 44                          | 40                          | 10.5                        | 0.187                        | 0.104                        | 4.2                                                                 | 1.6  |

cooled to room temperature after another 11 minutes.

The measured results obtained in the resulting rings are again recorded in the table after Example V.

#### EXAMPLE III

The composition of the starting mixture was as follows:

|                                | Mol percent |
|--------------------------------|-------------|
| Fe <sub>2</sub> O <sub>3</sub> | 77.21       |
| Li <sub>2</sub> O              | 13.61       |
| ZnO                            | 3.13        |
| NiO                            | 6.05        |

For sintering the rings (which had an outside diameter of approximately 0.5 mm. and an inside diameter of approximately 0.3 mm.) the platinum boat that the rings was again arranged in the course of 30 seconds in the hottest furnace region where a temperature of approximately 1175° C. prevailed. Four minutes later the boat with the rings was pulled out of the furnace at a substantially constant speed in such manner that the rings were cooled to room temperature after approximately another 9 minutes.

The measured results of the resulting rings are again recorded in the table after Example V.

What is claimed is:

1. A method of manufacturing a magnet core suitable for use as a memory element in electronic computers comprising the steps of forming a mixture of:

74.5—80.0 mol percent Fe<sub>2</sub>O<sub>3</sub>

12.5—14.6 mol percent Li<sub>2</sub>O

3.0—8.0 mol percent of ZnO

and up to 6.1 mol percent NiO,

preparing and compacting said mixture into annular bodies, raising the temperature to said bodies in a heating zone to between 1100° C. and 1200° C. within one minute, maintaining said bodies in said heating zone at said temperature for approximately 1½ to 8 minutes, and thereafter gradually withdrawing said bodies from said heating zone at a substantially constant speed to cool said bodies to room temperature in about 5 to 30 minutes.

2. A method as claimed in claim 1 wherein the bodies are heated to said temperature in 30 seconds.

3. A method as claimed in claim 1 wherein said bodies are cooled to room temperature in 8 to 20 minutes.

## References Cited

## UNITED STATES PATENTS

3,293,184 12/1966 Van Driel et al. ---- 252—62.61  
3,038,860 6/1962 Vinal et al. ----- 252—62.61  
3,226,328 12/1965 Esvedt et al. ----- 252—62.61  
3,370,011 2/1968 Kitagawa et al. ---- 252—62.61  
3,637,504 1/1972 Schmid ----- 252—62.61

## FOREIGN PATENTS

626,825 7/1963 Belgium ----- 252—62.61  
1,012,814 12/1965 Great Britain ----- 252—62.61  
165,254 1/1963 U.S.S.R. ----- 252—62.61

5 ROBERT D. EDMONDS, Primary Examiner

U.S. CL. X.R.

752—62.62